

June 2, 1931.

E. R. CLARK

1,808,593

MANUFACTURE OF FLAX FIBER

Filed Aug. 17, 1927

2 Sheets-Sheet 1

FIG. 1A.



FIG. 1.

INVENTOR

Edgar R. Clark

BY

Pennie, Davis, Marin & Edwards  
ATTORNEYS

June 2, 1931.

E. R. CLARK

1,808,593

MANUFACTURE OF FLAX FIBER

Filed Aug. 17, 1927

2 Sheets-Sheet 2



INVENTOR

Edgar R. Clark

BY

Pennie, Rain, Marion & Edwards  
ATTORNEYS

## UNITED STATES PATENT OFFICE

EDGAR RAYMOND CLARK, OF PITTSBURGH, PENNSYLVANIA, ASSIGNOR TO MILTON S. ERLANGER, OF NEW YORK, N. Y.

## MANUFACTURE OF FLAX FIBER

Application filed August 17, 1927. Serial No. 213,511.

This invention relates to improvements in the manufacture of flax fiber, more particularly to improvements in the manufacture of flax fiber from seed flax straw.

5 Although several million acres are planted annually to flax in the United States at present, only a fraction of one per cent of this acreage produces flax available for the production of commercial flax fiber; the 10 ponderance of the flax is grown for seed. There are at least two reasons for this situation—the wage standard in the United States, when present methods are used, almost precludes competition with foreign 15 sources of flax fiber and the cultivation of flax for fiber is not entirely consistent with the production of a high yield of good quality seed. As a result there is a large annual production of seed flax straw which has not been 20 available for the production of a high grade flax fiber. Some of this seed flax straw is used in the manufacture of coarse yarns, some of it is used in the manufacture of a "tow" used in upholstering but not of a form suitable 25 for spinning, some of it is used in the manufacture of a pulp employed in thermal insulation, but much of it is burned as a waste product.

This invention provides an improved method of manufacturing flax fiber from seed flax straw. The invention makes it possible, for example, to manufacture from seed flax straw a flax fiber suitable for spinning high grade tow yarns or a flax fiber product the equal of 35 linen rags for the production of paper or a high grade absorbent fiber product, at commercially feasible costs. The invention, however, includes several improvements of general utility in the manufacture of flax fiber.

40 The complete process of the invention comprises, first, a special retting operation, second, a special drying of the retted material, third, a special towing operation, and, fourth, 45 a further cleaning operation adapted to the particular purpose for which the fiber is manufactured. The sequence and combination of the several particular operations which make up the complete process of the 50 invention have several important advantages.

The invention, however, also includes improvements in the individual operations.

The invention relates particularly to improvements in the manufacture of flax fiber from seed flax straw, and will be further described more particularly as applied to the treatment of seed flax straw, but it will be understood that the invention includes features of more general application.

The accompanying drawings illustrate, 60 diagrammatically and conventionally, apparatus adapted for carrying out the process of the invention. In the accompanying drawings, Fig. 1 illustrates a retting tank with associated apparatus; Fig. 1A represents a 65 modified form of heating means for use in connection with the apparatus illustrated in Fig. 1; Fig. 2 represents an improved towing machine adapted for carrying out the special towing operation of the invention; Fig. 3A 70 represents a conventional cotton carding machine, and Fig. 3B represents a conventional flax tow-carding machine.

Seed flax straw is usually collected in bales. Before the straw is subjected to the improved 75 retting operation of the present invention, such bales are opened and any seeds left over from the threshing operation, as well as any residual chaff and adventitious matter without fiber value, are separated from the straw. 80

The straw is then packed in large tanks equipped with suitable means for maintaining circulation of the retting liquor through the tank and through some appropriate external heating means. The capacity of the 85 tank, advantageously, should be such as to make possible a straw to water ratio in the neighborhood of from 1:10 to 1:12 with a moderate degree of compression.

Fig. 1 illustrates one form of apparatus which may be used for carrying out the retting operation. The apparatus there illustrated comprises a tank 4 provided with a screen 5 spaced some distance above the bottom and with a loose screen 6 adapted to rest on top of the straw packed in the tank. Connections 7, 8 and 9, including circulating pump 10, are arranged to maintain circulation of retting liquor through the tank and through the straw packed therein. The heat- 95 100

er 11 is arranged in the circulating connections for raising the retting liquor to and maintaining it at the desired temperature. This heater, for example, may be a shell and tube heater as illustrated in Fig. 1 or the circulating liquor may be heated directly by the introduction of steam through a suitable injector 12, as illustrated in Fig. 1A. Connection 13 is provided for discharging liquor from the tank and connection 14 for supplying liquor to the tank, and appropriate valves are provided, as illustrated, for regulating the supply, discharge and recirculation of the liquor.

15 The retting operation proper is advantageously carried out at a temperature of about 30° C. and the circulation of the retting liquor is advantageously maintained at a rate such that the entire volume of the liquor circulates through the tank, or through the external circuit including the heating means, not less than about once per hour or better, not less than about twice per hour. The flax straw is advantageously rinsed in 20 the retting tank with cold water both before and after the retting operation proper, and following retting, the straw may, with advantage, be drained before removal from the tank.

25 30 In a typical operation, the retting tank is packed with seed flax straw and the straw is wet down with about 400 gallons of water for every 300 pounds of straw. Cold water, say at a temperature of from 5 to 20° C., is used 35 in this operation. This preliminary wash water is circulated through the tank several times; this preliminary washing, including the filling and draining of the tank, may take, for example, about 3 hours. In addition 40 to thoroughly wetting the straw, this preliminary washing assists in removing loose dirt and a certain portion of carbohydrate matter. In many cases, this preliminary washing is of material assistance in making 45 the resulting fiber product more easily and more effectively bleached.

50 After this preliminary washing, about the same quantity of water is again supplied to the retting tank and gradually raised to the 55 temperature required for the retting operation, about 30° C. Fermentation begins soon after this refilling of the tank and warming of its liquid contents. The desirable type of fermentation is accelerated by the preliminary removal or partial removal of any readily 60 fermentable sugars. These in fermenting give rise to acid products inhibitory to the action of the true retting bacteria. The retting liquor is maintained in circulation 65 through the retting tank and through the external heating means throughout the operation and is thereby maintained at a substantially uniform temperature. This circulation of the retting liquor not only promotes 70 uniformity but also makes the retting opera-

tion readily amenable to control. Usually, the seed flax straw is satisfactorily retted after about 45 hours of treatment at elevated temperatures. Reducing sugars usually disappear about 21 hours after the warming of the retted liquor. During the remainder of the retting period, while the fermentation of pectin is proceeding, the acidity of the retted liquor is advantageously maintained approximately at pH=6.0. 75

When the retting operation proper is completed, the retted liquor is drained off and about the same quantity of water is again supplied to the retting tank. This wash water is circulated through the tank several times and is then drained from the tank. The retted straw is then removed and subjected to a suitable drying operation. 80

With the improved control and uniformity provided by the improved retting operation of this invention, the operation can be terminated, for all practical purposes, by the clock once the appropriate period for the particular type and condition of straw handled is determined. The end point of the retting operation can best be determined by noting the brittleness of the woody matter of the flax. This feature of the invention minimizes danger of overretting which makes for tenderness as well as danger of underretting, which prevents satisfactory scutching. The retting process of this invention, moreover, can be carried on without reference to the season of the year. 95

100 The moist or damp flax straw from the retting operation may be dried in a variety of ways; but the drying is advantageously carried out at temperatures which do not at any time during the drying operation exceed about 60° C., to avoid the premature swelling of the pectinous matter of flax and its setting to a permanent stiffened form. Flax dried at too high a temperature is unsuited to the finer forms of spinning, particularly wet spinning. By maintaining the temperatures during drying below this value, the quality of the flax fiber produced is much enhanced. It is also advantageous to reduce the temperature to about 35° C. or less as soon as the straw becomes sensibly dry to 105 avoid any loss of moisture and oily elements necessary for suppleness. This drying can be carried out in any convenient form of apparatus. 110

115 In carrying out the complete process of the invention, the dry, retted flax is then subjected to a special towing operation to straighten and open the fiber, to break up tangles, and to separate the shives. An apparatus adapted for carrying out this special 120 towing operation is illustrated in Fig. 2.

125 Referring to Fig. 2, the flax passes first between a series of pairs of fluted breaking rolls 15 where it is subjected to a breaking operation. These breaking rolls are in them- 130

selves of conventional construction and operation. From these breaking rolls, the flax is delivered between a pair of toothed lattices 16 and 17 by means of a traveling apron 18. A stripping brush may be arranged as illustrated. The lower lattice 16 is carried by rotating supports 18 and 19 and the upper lattice 17 is carried by rotating supports 20 and 21. These rotating supports for the lattices 16 and 17 are arranged so that the co-operating portions of the lattices move in substantially parallel planes. The lattices are driven in the same direction. The teeth on the lower lattice are inclined toward the direction of motion of the lattice and the teeth on the upper lattice are inclined against the direction of motion of the lattice. The lower lattice 16 is driven at a speed sufficiently greater than that of the upper lattice 17 so that the draft in passing between the lattices exceeds the maximum fiber length. These lattices may comprise, for example, teeth mounted in slats, the slats in turn being carried at each end by sprocket chains. A doffing wheel 22, for example, a bristle or wire covered wheel, is arranged to remove fiber from the lattice 16. The rotating support 21 is advantageously arranged, as illustrated, so that the upper lattice 17 moves away from the lower lattice 16 before the lower lattice leaves the plane of its travel in cooperation with the upper lattice. The doffing wheel 22 is advantageously driven at a speed such that the velocity at the periphery is somewhat greater, say 5%, than the velocity of the lattice 16.

From the doffing wheel 22, the flax is again delivered to a series of pairs of breaking rolls 15a or to a shaking mechanism 23 adapted to subject the flax to a tossing action or the flax may be passed successively through breaking rolls and over such shaking mechanism. By means of another traveling apron 18a, the flax may then be delivered between another pair of lattices similar to 16 and 17 and thence through another series of pairs of breaking rolls similar to 15a and then over a shaking mechanism similar to 23, and so on, any desired or required number of times. For example, the flax, after passing through a series of pairs of preliminary breaking rolls, such as 15, may be passed three times in succession through the apparatus illustrated between the apron 18 and the point 55 designated C in Fig. 1 and finally discharged through a pair of lattices 16c and 17c similar to lattices 16 and 17. The breaking rolls following the doffing wheels, for example, the breaking rolls 15a following doffing wheel 22, are advantageously driven at a speed such that the peripheral velocity of the breaking rolls is a little greater than that of the doffing wheel with which they cooperate.

The operation carried out by means of the lattices 16 and 17, and by the doffing wheel

22, is of special value in towing flax. It effects a special cleaning and straightening and provides positive doffing, even where the fiber length varies excessively.

The particular towing operation just described is, moreover, of special value and application in conjunction with the particular retting operation previously described. The combined result of this particular retting operation and this particular towing operation is the production of a fiber stock readily adaptable to carding and spinning or other operations for the manufacture of textiles, paper, absorbents, and the like. The retting process of the invention is rapid and controllable and is adapted to large scale factory operation and at the same time brings the flax to condition such that, by means of the special towing operation of the invention, a satisfactory flax fiber can be produced simply and economically.

In the manufacture of textiles, the flax fiber is then ready for carding in the usual way, the carding operation starting the formation of the sliver for spinning. The spinning can then be carried out on the usual flax machinery.

In the manufacture of paper, the fiber from the special towing operation of the invention is advantageously processed in a cotton carding machine for complete separation of shives. The presence of shives in flax fiber prohibits the manufacture of a readily bleachable paper pulp by the alkaline processes of digestion to which such fiber is naturally adapted; but, by substantially complete removal of shives by this invention, such cooking processes yield an easily bleachable pulp. By thus finishing the cleaning of the flax fiber product from the special towing operation of the invention, after retting in accordance with the invention, a flax fiber can be obtained which is essentially pure flax and which is substantially the equal of unbleached linen rags for the manufacture of paper. This fiber product may be bleached and is then substantially the equal of bleached linen rags for the manufacture of paper.

A conventional cotton-carding machine adapted for carrying out such further cleaning of the improved tow of the invention is diagrammatically illustrated in Fig. 3A. It comprises a licking-in wheel 24 by which the tow is fed to the carding drum 25 over which the lattice 26 moves, the lattice 26 moving in the same direction but at a slightly lower velocity than the periphery of the drum 25, and a doffing wheel 34.

Instead of processing the fiber from the special towing operation of the invention in a cotton carding machine, it may be processed on a flax-tow-carding machine, a conventional machine adapted to this purpose being diagrammatically illustrated in Fig. 3B. It comprises a pair of feed rolls 27 by which

the tow is supplied to the carding drum 28. A series of cooperating pairs of working rolls 29 and doffing rolls 30 are arranged about the periphery of the drum 28. The carding elements on the drum 28 are inclined in the direction of motion. The periphery of the carding drum 28 is driven in the same direction as the cooperating portion of the periphery of the rolls 29 and wheels 30. The carding elements on the working rolls 29 are inclined against the direction of motion and the doffing elements on the wheels 30 are inclined toward the direction of motion. The working rolls 29 are driven at a speed such that the peripheral velocity is somewhat less than that of the carding drum 28. The carded fiber may be removed from the carding drum by a series of doffing wheels 31, 32 and 33; the successive doffing wheels each being arranged closer to the axis of the carding drum.

The fiber product produced by processing on the flax tow-carding machine is similar to that produced by processing on the cotton carding machine but of longer fiber. The operation is less expensive than processing on the cotton card as the latter requires that the stock be first prepared in a lap form, in the usual way, requiring additional time and labor. The cotton card processing effects however a more complete removal of shives, and the flax tow card is ordinarily used only for making spinning fiber, or grades of paper in which the complete removal of shives is not essential. The flax tow card yields a fiber product better adapted to the usual bleaching and purifying operations employed in making absorbent fiber, than does the cotton card.

Whether the final cleaning operation is carried out on a cotton-carding machine or a flax tow-carding machine, or otherwise, the complete process of the invention including the special retting operation, the special towing operation and this carding, makes possible the production from seed flax straw of a flax fiber product which is free from shives, which is extremely clean, and which is of quality comparable to the common grades of tow produced from flax grown for fiber.

This invention also includes improvements in apparatus for carrying out the special towing operation of the invention. The apparatus illustrated, diagrammatically and conventionally, in Fig. 2 embodies this aspect of the invention.

I claim:

1. In retting flax, the improvement which comprises placing the flax in a tank, rinsing the flax in the tank by circulating cold water therethrough and, after draining off the rinsing water, supplying fresh water to the tank and maintaining it at a uniform elevated temperature by circulating it from the tank through an external circuit back to the

tank and heating it while passing through the external circuit.

2. In drying flax subsequent to a retting operation, the improvement which comprises conducting the drying at temperatures higher than ordinary field drying temperature but not exceeding 60° C. throughout the drying operation.

3. In drying flax subsequent to a retting operation, the improvement which comprises drying the flax at an initially elevated temperature and reducing the temperature as the drying proceeds, the entire drying operation being conducted at temperatures not exceeding 60° C.

4. In retting flax, the improvement which comprises washing the flax straw with cool water, removing the wash water from the flax, submerging the flax in fresh water in a closed container, uniformly heating the water to a temperature of about 30° C., circulating the water throughout the container so as to maintain uniformity of conditions affecting the fermentation, removing the water when the retting has reached the desired degree, and drying the flax at a temperature below about 60° C.

5. The process according to claim 4 in which the container during the fermentation is completely filled with straw and water in the ratio of about one part of straw to ten parts of water.

6. The process according to claim 4 in which the bath is maintained at the desired temperature by circulating it through an external heating means.

7. The process according to claim 4 in which uniform conditions are maintained throughout the bath by passing its entire volume through a suitable circulating means at least once per hour.

8. The process according to claim 4 in which the bath is maintained during the fermentation of the pectin at an acidity of about pH 6.0.

9. The process according to claim 4 in which the temperature of the drying operation does not exceed about 35° C. after the straw has become sensibly dry.

10. The process according to claim 4 in which the straw is rinsed with fresh water after the fermentation and before drying.

11. In retting flax, the improvement which comprises maintaining the material at an acidity of about pH 6.0 during the fermentation of the pectin.

12. In retting flax, the improvement which comprises maintaining the material uniformly at an acidity of about pH 6.0 and a temperature of about 30° C. throughout the desired fermentation of the pectin.

13. In drying flax subsequent to a retting operation, the improvement which comprises drying the flax at an initially high temperature, said initial temperature exceeding 35°

C. but not exceeding 60° C., maintaining said initial temperature until the material is sensibly dry, then lowering the temperature and completing the drying at a temperature not lower than about 35° C.

5 14. In the manufacture of flax fiber wherein said fiber is subjected to retting, drying and scutching operations, the improvement which comprises drying the retted straw at 10 a temperature maintained between 60° C. and 35° C.

15 15. In the manufacture of flax fiber wherein said fiber is subjected to retting, drying and scutching operations, the improvement which comprises drying the flax at an initially higher temperature, said initial temperature exceeding 35° C. but not exceeding 60° C., maintaining said initial temperature until the material is sensibly dry, then lowering the temperature and completing the drying at a temperature not lower than about 20 35° C.

In testimony whereof I affix my signature.  
EDGAR RAYMOND CLARK.

25

30

35

40

45

50

55

60

65